



US006040032A

# United States Patent [19]

Isräel et al.

[11] Patent Number: 6,040,032

[45] Date of Patent: Mar. 21, 2000

- [54] **ABSORBENT ARTICLE FOR COLLECTING  
NON-AQUEOUS LIQUIDS AND A METHOD  
FOR MANUFACTURING THE ABSORBENT  
ARTICLE**

- 4,747,960 5/1988 Freeman et al. ..... 210/689  
 4,784,773 11/1988 Sandberg ..... 210/691  
 5,009,790 4/1991 Bustamante ..... 210/689

- [76] Inventors: **Joseph Israël**, 111 Old Bay Rd., Belchertown, Mass. 01007; **Yvon Levesque**, 3103 St. Catherine, Montreal, Quebec, Canada, H1W 2E6

## FOREIGN PATENT DOCUMENTS

- [21] Appl. No.: 08/054,448

- [22] Filed: Apr. 28, 1993

- [51] **Int. Cl.<sup>7</sup>** ..... **B32B 5/00**; B32B 9/04;  
B27N 3/00

- [52] U.S. Cl. .... 428/98; 264/109; 428/411.1;  
502/401

- [58] **Field of Search** ..... 210/611, 622,  
210/682; 435/262.5; 252/610, 301; 502/402,  
401; 428/98, 411.1; 264/1099

[56] **References Cited**

## U.S. PATENT DOCUMENTS

- |           |        |               |         |
|-----------|--------|---------------|---------|
| 3,791,990 | 2/1974 | Fischer ..... | 252/427 |
| 4,497,712 | 2/1985 | Cowling ..... | 210/691 |

*Primary Examiner*—Wayne Langel  
*Attorney, Agent, or Firm*—James P. Barr

[57] ABSTRACT

An absorbent article for collecting non-aqueous liquids such as oil-based products, comprising a low density, structurally integral board of peat moss material manifesting an affinity for non-aqueous liquids while being hydrophobic in order to block undesirable water penetration in the absorbent medium. The invention also extends to a method for manufacturing the absorbent article.

**20 Claims, 3 Drawing Sheets**





FIG.1



FIG.2



FIG. 3

**ABSORBENT ARTICLE FOR COLLECTING  
NON-AQUEOUS LIQUIDS AND A METHOD  
FOR MANUFACTURING THE ABSORBENT  
ARTICLE**

**FIELD OF THE INVENTION**

The invention relates to the general field of spill management and, more particularly, to a novel absorbent article utilizing peat moss material for collecting non-aqueous liquids such as oil-based products. The invention also extends to a method for manufacturing the absorbent article.

**BACKGROUND OF THE INVENTION**

The prior art has recognized the potential of peat moss material for use as an absorbent medium in structures for absorbing aqueous solutions. The remarkable fluid absorption properties of peat moss material have been turned to use in the field of sanitary, disposable absorbent products such as sanitary napkins, tampons, diapers, adult briefs, urinary pads, wound dressings and the like, to provide highly efficient absorbent components which can be made relatively thin for better fit, comfort and discretion, while being sufficiently absorbent to prevent overflow leakage of body exudate and garment staining.

The following United States patents document the use of peat moss material for manufacturing absorbent components for sanitary, disposable absorbent products.

| U.S. Pat. No. | INVENTOR(S)       | DATE OF ISSUE      |
|---------------|-------------------|--------------------|
| 4,170,515     | Lalancette et al. | October 9, 1979    |
| 4,215,692     | Levesque          | August 5, 1980     |
| 4,226,237     | Levesque          | October 7, 1980    |
| 4,305,393     | Nguyen            | December 15, 1981  |
| 4,473,440     | Ovans             | September 25, 1984 |
| 4,507,122     | Levesque          | March 26, 1985     |
| 4,618,496     | Brasseur          | October 21, 1986   |
| 4,676,871     | Cadieux et al.    | June 30, 1987      |
| 4,992,324     | Dube              | February 12, 1991  |
| 5,053,029     | Yang              | October 1, 1991    |

The subject matter of these patents is incorporated herein by reference.

Peat moss material can be formed in a highly cohesive, structurally integral board by any one of the methods disclosed in the above-identified prior art. In board form, the absorbent material is more convenient to handle and it can be directly processed in high speed automatic equipment for assembling disposable absorbent products.

Broadly stated, the method developed by the industry for manufacturing a structurally integral peat moss board which is specifically adapted for sanitary usage, comprises the following steps. Raw peat moss, in particulate form, is classified by wet screening in order to retain only the particles which are the most absorbent. The screened fraction is diluted with water to form a slurry having a pumpable consistency which is sheeted on a Fourdrinier wire and dewatered by the sequential application of vacuum and heat. The thus formed board is calendered at high pressure to increase its density primarily for the purpose of enhancing its drying power, i.e. the ability of the absorbent medium to continuously pull and wick fluid away from adjacent materials such that virtually all the fluid is collected in the peat moss core. This consideration is particularly important for sanitary absorbent products which are intended to remain in contact with the skin of the wearer for an appreciable period

of time. In such applications, the capability of the peat moss core to extract moisture from the fluid permeable cover of the sanitary product which receives the discharge of body exudate is a highly desirable attribute as it allows to impart to the fluid permeable cover a feeling of "dryness" which makes the absorbent product more comfortable to wear.

During the formation stage of the peat moss board, the aqueous slurry is treated with a wetting agent (hereinafter "wetting agent" shall be construed to encompass any substance which imparts hydrophilicity or enhances the hydrophilicity of the peat moss material), such as a surfactant, to provide the peat moss board with a strong affinity for water. Typically, the wetting agent is added to the peat moss slurry at the vacuum dewatering stage by spraying or by any other appropriate deposition method. The pressure differential established across the Fourdrinier wire to extract dilution water constitutes the agency which causes the wetting agent to penetrate deeply in the peat moss slurry.

The prior art also recognizes the efficiency of peat moss material to absorb non-aqueous liquids such as a variety of chemical products and specifically oil-based materials. The waste management industry has been using peat moss as an absorbent medium for the removal of non-aqueous, liquid pollutants, for many years. Typically, dried particulate peat moss packaged into liquid permeable pouches is delivered to the contaminated area and placed in contact with the liquid spill to absorb the pollutant. By virtue of the relatively low density of peat moss material in particulate form, the absorbent pads have the ability to float on water and can be used for recovering non-aqueous, liquid pollutants floating on a body of water, such as an oil slick on sea surface for example.

Although particulate peat moss material has the ability to collect and trap many times its own weight of oil-based products and a variety of other chemicals, the configuration of the absorbent pads made from this material is not well suited for the recovery of large scale spills. Granular peat moss material has virtually no structural integrity, and when it is loaded into a flexible containment pouch, the resulting absorbent pad assumes the shape of a bag, i.e. a bulbous round body in which the ratio outer surface/volume is relatively low. As a result, the liquid take-up rate is low which requires a longer residence time of the absorbent pad in the spill in order to reach the saturation level. This drawback is particularly significant for applications where the absorbent pad is subjected in use to vigorous movements by natural forces, such as sea waves or wind, having a tendency to separate the absorbent pad from the spill. In such applications a high fluid take-up rate is highly desirable to allow an efficient utilization of the available absorbent material.

Having regard to the foregoing, a primary objective when designing an absorbent pad for spill management purposes should be to attain the broadest possible outer surface in order to increase the contact surface with the liquid pollutant and therefore to enhance the liquid take-up rate. A suitable shape would be a sheet-like or a board-like configuration which is characterized by a broad outer surface and little thickness.

However, granular peat moss material which is currently used by the industry is unsuitable for making board-shaped absorbent pads because it has little or no ability to maintain a predetermined shape, unless one uses a liquid permeable pouch which cumulates the functions of a containment envelope and of a structural member to impart to the absorbent material a certain shape. However, for cost considerations, this option is unpractical.

To compensate for the limited outer surface of conventional absorbent pads, one may use a larger number of pads for a given amount of liquid pollutant. The drawback behind this approach is twofold. Firstly, a larger number of absorbent pads makes the recovery operation more expensive. Secondly, this practice, in itself, may create an environmental hazard because the pouches used to contain the loose peat moss material are made from a non-biodegradable plastic such as a non-woven polyester fabric, therefore if some absorbent pads drift away during the recovery operation and are lost they will contaminate the environment.

It has also been suggested in the past to apply peat moss material to the liquid pollutant in particulate form and subsequently to recover the peat moss material with the liquid pollutant trapped therein. This method avoids the difficulties associated with absorbent pads made of granular peat moss material packaged in liquid permeable pouches, however, this use is restricted only to land or hard surfaces and on spills of limited extend. Loose peat moss material cannot be practically used for large-scale spills on land or on water because the recovery of the spent absorbent is strenuous and costly due to its particulate nature.

#### OBJECTS OF THE INVENTION

An object of the invention is to provide an absorbent article for collecting non-aqueous liquids, such as oil-based products and a variety of other chemicals, utilizing peat moss material as an absorbent medium, which is relatively inexpensive and simple to produce and which has a comparatively broad exterior surface providing a high fluid take-up rate.

An underlying object of the invention is an absorbent article having the above stated properties and which is also buoyant, thereby being capable of recovering liquids floating on a body of water.

Another object of the invention is a method for manufacturing the aforementioned absorbent article.

#### SUMMARY OF THE INVENTION

The present inventors have made the unexpected discovery that peat moss material formed into a hydrophobic, structurally integral board (hereinafter, the term "board" is intended to encompass sheet-shaped objects which are not necessarily rigid, such as a flexible mat) provides an absorbent article suitable for recovering a large variety of non-aqueous liquids, which is relatively simple and inexpensive to mass produce and it is characterized by an exceptional absorbent capacity and a high liquid take-up rate. A significant advantage of the invention over the prior art resides in that the peat moss board does not require a discrete, confining structure, such as the liquid-permeable pouch used in traditional absorbent pads. This results into a cost-effective, environmentally sound absorbent article.

Experimental work conducted on the absorbent article in accordance with the invention has demonstrated a definite correlation between the density of the peat moss board and its absorbent capacity. More specifically, it has been established that by decreasing the density of the peat moss board, its absorbent capacity increases.

It is important to note that the density of the peat moss board also influences its strength and resistance characteristics. Therefore, a very low density board, albeit having a very high absorption capacity, is not necessarily desirable because it may be subject to structural failures in operation, especially when the board becomes saturated with liquid.

A possible approach to increase the resistance of the peat moss board without significantly adding to its density is to use a laminated form of construction by bonding to the peat moss material one or more thin layers having a relatively high tensile strength.

In a preferred form of construction, the laminated peat moss board comprises an absorbent core of peat moss material sandwiched between thin layers of fibrous material such as Kraft wood pulp. In a preferred embodiment, the overall density of the structure is in the range from about 0.02 grams per cubic centimeter (g/cc) to about 0.20 g/cc (all density measurements provided in this specification are effected on samples at 12% moisture level). More preferably, the density is in the range from about 0.05 g/cc to about 0.15 g/cc. Most preferably, the density of the board is in the range from about 0.05 g/cc to about 0.10 g/cc.

A critical aspect of the invention is the ability of the peat moss board to shed water while being capable of absorbing non-aqueous liquids, such as oil-based products. Such selective absorption properties allow to provide an absorbent article which can be successfully used for recovering a non-aqueous liquid present into an environment containing a significant amount of water, for example an oil slick floating on sea surface. The low density of the peat moss board confers buoyancy to the absorbent article allowing same to float on the water surface exactly where the non-aqueous liquid is located. Further, the water repellency of the peat moss board prevents undesirable saturation of the absorbent article with water, thereby maintaining the absorbent medium active for capturing the non-aqueous liquid.

Throughout this specification, the peat moss board in accordance with the invention will be described as hydrophobic with reference to its ability to prevent ingress of water within the absorbent medium. This terminology takes into account only the general behaviour of the peat moss board and does not imply that each of its constituents has no affinity for water. For example, in the laminated form of construction described earlier utilizing an absorbent core of peat moss material sandwiched between thin layers of Kraft wood pulp, the peat moss board is not perfectly hydrophobic since the reinforcing Kraft pulp layers are capable of some water absorption which, however, is minimal and can be disregarded in practice. In such exemplary form of construction, when a small amount of water is deposited on the outer surface of the absorbent article, the water will penetrate within the Kraft wood pulp layer, however, it will be arrested therein and it will not be able to propagate within the absorbent core. Therefore, the saturation level to water of the absorbent article is extremely low and does not affect its selective absorption properties in any significant way.

It will be plain to a person skilled in the art that the hydrophobicity of the peat moss board can be perfected by treating the Kraft wood pulp layers with a suitable water repelling agent.

As embodied and broadly described herein, the invention also extends to an absorbent article for recovering an oil-based liquid floating on a body of water, the absorbent article including a structurally integral and buoyant board of peat moss material, the board of peat moss material being hydrophobic and oleophilic, whereby when the board of peat moss material is floated on the body of water in contact with the oil-based liquid, the board of peat moss material selectively absorbs the oil-based liquid without taking-up any significant amount of water.

As embodied and broadly described herein, the invention also extends to a method for manufacturing a low density,

structurally integral article for collecting non-aqueous liquids, the method comprising the steps of:

- a) forming a liquid suspension of peat moss material;
- b) sheeting the suspension;
- c) extracting fluidizing medium from the suspension to form a low density board of peat moss material;
- d) drying the board of peat moss material;

the method being completed without conditioning the peat moss material with wetting agent to preserve a natural hydrophobicity of the peat moss material in order to impede water penetration in the article.

In a most preferred embodiment, raw peat moss material is formed into an aqueous slurry having a pumpable consistency and it is subjected to a classification procedure to eliminate from the peat moss slurry particles having a size substantially smaller than 210 microns and particles having a size substantially larger than 2000 microns, in order to retain only the particles which are the most absorbent. The peat moss slurry is classified by flowing the slurry through a set of screens having the desired mesh size.

The slurry is then delivered on a Fourdrinier wire and dewatered by the sequential application of vacuum and heat to form the absorbent article. If desired, the article may be calendered at a very low pressure solely for the purpose of stabilizing its calliper. Intense calendering is to be avoided because it would have the effect of increasing the density of the peat moss material which adversely affects its absorption capacity.

To manufacture a laminated peat moss board of the type described earlier, a co-forming process may be used which consists of progressively building on the Fourdrinier wire a stratified slurry by successive deposition of water suspension strata corresponding to each layer of the final product.

#### BRIEF DESCRIPTION OF THE DRAWINGS

FIG. 1 is a perspective, fragmentary view of an absorbent article constructed in accordance with the present invention;

FIG. 2 is a schematical representation of an apparatus for manufacturing the absorbent article shown in FIG. 1; and

FIG. 3 is a graphical representation of the relationship between the density of the absorbent article and its absorption capacity, for various types of non-aqueous liquids.

#### DESCRIPTION OF PREFERRED EMBODIMENTS

The structure of an absorbent article constructed in accordance with the present invention which can be used for recovering non-aqueous liquids is illustrated in FIG. 1. The absorbent article, designated comprehensively by the reference numeral 10, has a laminated structure and it is in a form of a relatively flat board comprising a central absorbent core 12 containing primarily peat moss material. The core 12 is confined between reinforcing layers 14 and 16 of fibrous material. The purpose of the reinforcing layers 14 and 16 is to strengthen the absorbent core 12, thereby providing a unitized absorbent structure capable of maintaining its integrity even when saturated with liquid. Kraft wood pulp material has been found highly satisfactory for manufacturing the reinforcing layers 14 and 16. It is also possible to use cotton linters or ground wood in admixture with or in substitution to the Kraft wood pulp material.

The detailed composition of the absorbent article 10 will be best understood from the following description of the apparatus and the process for manufacturing such absorbent

article. Referring to FIG. 2, the apparatus designated comprehensively by the reference numeral 18, comprises an endless, fluid-pervious Fourdrinier wire 20 which is mounted on rollers 22 to provide a horizontally extending run 24 which is continuously advanced forward to support and convey a slurry of peat moss material and Kraft wood pulp through various processing stations.

Headboxes 26, 28 and 30 arranged in a spaced apart relationship along the path of travel of the wire 20, are provided to lay on the wire 20 slurry in sheeted form. The headbox trio deposits on the wire 20 three layers of slurry in a superposed relationship to form a laminated web. More specifically, the central headbox 28 lays a slurry of peat moss and the headboxes 26 and 30 deliver slurry of fibrous material such as Kraft wood pulp or any other suitable substance.

The peat moss slurry, before being supplied to the headbox 28 is refined at a screening station illustrated schematically in FIG. 2 and identified by the reference numeral 32. The screening station 32 is of a well-known construction and does not require a detailed description herein.

Downstream of the headboxes 26, 28 and 30 is provided a vacuum slot 34 which is in fluid communication with a vacuum pump (not shown in the drawings) in order to create suction beneath the wire 20 for dewatering the slurry thereon.

The next processing station is dryer 36 whose purpose is to elevate the temperature of the slurry to evaporate water therefrom. The dryer is of a well-known construction and does not require a detailed description herein.

Downstream of the dryer 36 is provided a calendering station 38 which slightly compresses the dried product in order to stabilize its calliper.

The operation of the apparatus 18 is as follows. The starting peat moss harvested from the bog should have a relatively high absorbent capacity. Peat moss capable of absorbing and retaining at least about 25 and preferably about 50 times its weight in water has been found satisfactory. The starting peat moss is wet classified at the screening station 32 to remove the extremely fine material, commonly referred to as fines, and large pieces of material including roots, branches and the like which do not contribute significantly to the absorbency of the peat moss material.

The classification is carried out such that anything that remains on a number 10 mesh screen (2000 microns) is discarded and anything that passes through a number 70 mesh screen (210 microns) is also discarded. Preferably, anything that remains on a number 14 mesh screen (1410 microns) is discarded and anything that passes through a number 100 mesh screen (149 microns) is discarded.

The peat moss material is classified by a well-known wet screening process which consists of forming an aqueous slurry of the peat moss material and flowing the slurry through successive screens to extract from the slurry the fines and the excessively large particles.

The screened fraction of the peat moss material is then diluted with water to render the slurry more manageable. If desired, a fibrous component may be added at this stage to the slurry. The fibrous component may include such materials as Kraft wood pulp, mechanical wood pulp, cotton linters or jute, among others. As used herein, the term mechanical wood pulp is meant to include ground wood pulp, thermo-mechanical pulp and refiner wood pulp. Ground wood pulp is essentially trees and branches which have been debarked, cleaned and ground into particulate matter. Refiner wood pulp differs from ground wood pulp

only in that the grinding step utilizes a refiner, i.e. a disk-like device well-known in the art and having metallic ribs at the peripheral sections thereof which last contact the wood particles and help separate the wood fibers without excessively damaging them. Thermo-mechanical wood pulp is similar to refiner pulp with the exception that the wood particles are heated in the refiner, usually with steam, to aid in separating the wood fibers. The common characteristic of these mechanical pulps is that no attempt has been made to separate the fibers by chemical means although they may later, after being reduced to fine particulate matter, be subjected to a desired chemical treatment, such as bleaching.

Preferably, when mechanical wood pulp is used in the peat moss slurry, such mechanical pulp has a Canadian Standard Freeness (TAPPI TEST METHOD T-227) of from about 60 to 750 and preferably from about 400 to 600.

The Kraft wood pulp, also usable in combination with the peat moss, is essentially chemically treated, long fibred wood pulp such as sulfite and sulfate wood pulps.

The fibrous component may also include a natural or synthetic textile fiber such as rayon, polyester, nylon, acrylic or the like, having a length of from about 0.6 centimeters to about 1.9 centimeters, preferably about 1.3 centimeters and a denier of from about 1.0 to 5.0, present in an amount from 2 to 20% by weight of the absorbent core 12, preferably from 4% to 8%.

The slurry from the headboxes 26, 28 and 30 is sheeted onto the wire 20 and dewatered by the vacuum slot 34. If desired, a conditioning agent may be added to the slurry at this stage, such as a colouring agent, a water-repelling agent (for the purpose of this specification "water-repelling agent" should be construed to include any substance that procures hydrophobicity or enhances the hydrophobicity of the material to which it is applied) an adhesive or others. The selected conditioning agent may be applied to the slurry upstream of the vacuum slot 34 by spraying, coating or otherwise. The pressure differential established by the vacuum slot 34 causes the conditioning agent to penetrate within the peat moss and Kraft wood pulp compositions for an in-depth treatment.

The treatment of the slurry with water-repelling agent is particularly desirable in order to render the Kraft wood pulp layers hydrophobic. Various types of water-repelling agents can be used for the treatment. It is within the reach of the person skilled in the art to select the specific agent most suitable for the intended application.

After initial dewatering, the product is conveyed to the drier 36 for further dewatering by the application of heat. The thus formed board is slightly compressed at the calendering station 38 for stabilizing the calliper of the board.

It should be pointed out that the calendering of the laminated peat moss board is conducted at pressure levels significantly lower than the pressure developed when the peat moss board is intended for sanitary usage, where drying power should be enhanced by increasing the density of the absorbent medium. In contrast, for spill management purposes, a lower density is desired in order to increase the absorbent capacity of the peat moss board. Typically, the calendering pressure in the process according to the invention is about one tenth of the pressure which would be normally applied if the peat moss board was intended for sanitary applications.

After the calendering is completed, the continuous peat moss board is cut (this operation is not shown in the drawings) to form discrete absorbent articles having the desired size and shape. Preferably, the cutting pattern is

selected in such a way as to minimize waste. Square or rectangular shapes have been found satisfactory in this regard.

In a specific embodiment of this invention, a slurry of Kraft wood pulp having a consistency of about 0.2% by weight of solids is first laid down on the wire 20 from the headbox 26. The slurry flow rate is selected to deliver on the wire 20, 15 grams of solids per square meter. The Kraft slurry passes under the headbox 28 which delivers on top of the Kraft layer a slurry of peat moss material having the following composition by weight of solids:

Sphagnum peat moss  $\approx$  74.3%

Kraft wood pulp fibers  $\approx$  21.0%

Polyester fibers  $\approx$  4.7%

The consistency of the peat moss slurry is set at 0.5% by weight of solids. The flow rate of the peat moss slurry is selected to deliver 300 grams per square meter of solids on the wire 20.

A final Kraft wood pulp slurry layer is laid from the headbox 30 on the peat moss slurry. This final layer is identical in terms of consistency, flow rate and composition to the bottom Kraft wood pulp layer previously deposited.

The laminated slurry is passed over the vacuum slot 34 to extract water under the influence of a pressure differential established across the slurry. Precise regulation of the residence time of the slurry over the vacuum slot and the vacuum intensity is critical for accurate density control of the final product. Generally, decreased vacuum and increased speed will result in a less dense product.

Conversely, increased vacuum and decreased speed will produce a denser product. In a preferred embodiment, the speed of the wire 20 is set at 28.96 meters per minute. The vacuum slot 34 is constituted by a set of 6 elongated orifices which are parallel and are oriented transversely to the direction of travel of the wire 20. Each orifice has a width of 25.4 centimeters. Collectively, the orifices provide an interval of about 3 seconds during which the slurry is exposed to vacuum. The intensity of the vacuum ranges from about 200 to about 315 millimeters of mercury.

The dewatered product is then dried in the dryer 36 by subjecting the product to a temperature above 100° C. in order to evaporate residual moisture. The high temperature treatment is desirable because it has been found to enhance the hydrophobicity of the peat moss material.

Subsequently, the dried product is calendered at the calendering station 38 to control its calliper. A calendering pressure of approximately 275 kilograms per linear meter is used. The resulting laminated peat moss board has a density of 0.077 g/cc.

The calendering pressure applied on the peat moss board is dependent on the characteristics of the calendering equipment that is being employed. In other words, different calendering stations may develop exactly the same pressure at the nip, thus conditioning the calendered material in the same way, although the pressure reading in kilograms per linear meter is different for each station.

For the purpose of repeatability of the process conditions set forth herein, the calendering station that has been used to slightly compress the peat moss board has the following characteristics:

a) a top roll having a diameter of 42.929 centimeters, a length of 91.440 centimeters, a hardness of 75/82 shore C and a crown of 0.11557 millimeters; and

b) a bottom roll having a diameter of 45.664 centimeters, a hardness of 76/80 shore C and a crown of 0.10541 millimeters.

It should be appreciated that the calendaring operation enables the operator to control the density of the final product. However, this control lever is seldom used because it can only increase the density of the peat moss board which adversely affects its absorption capacity. Therefore, in practice, the calendaring station is set at the minimum pressure which will be sufficient to stabilize the calliper of the peat moss board.

A critical parameter of the process in accordance with the invention is that no attempt has been made to enhance the hydrophilicity of the peat moss board. This is contrary to conventional processes for the manufacture of peat moss boards, specifically designed for sanitary usage, where the absorbent medium must be capable of absorbing aqueous solutions. The preservation of the natural hydrophobicity of the peat moss material is an important characteristic of this invention which allows to produce an absorbent article capable of selective fluid absorption.

The following table considered in conjunction with the graph of FIG. 3, illustrates the relationship between the density of the laminated peat moss board and its absorbent capacity for various non-aqueous liquids. The table also provides a qualitative measure of the ability of the peat moss board to retain liquid absorbed in its structure. The various samples of peat moss boards considered in the comparative test have identical compositions, and weight and differ solely by their density. These samples have been produced by following the steps of the process set forth above, except that for samples B, C, D and E the calendaring pressure has been progressively increased in order to achieve a higher density. It should be appreciated that some of these samples, the most denser for instance, are not necessarily considered to be useful in practice due to their poor absorbency characteristics, and their purpose is only to illustrate the relationship between the density of the peat moss board and its absorbent capacity.

The description of the various test procedures to which the samples A, B, C, D and E have been subjected, are described in the section entitled "TEST PROCEDURES" following the table.

TABLE

| DENSITY (g/cc)                    | SAMPLES    |            |            |            |            |
|-----------------------------------|------------|------------|------------|------------|------------|
|                                   | A<br>0.077 | B<br>0.104 | C<br>0.176 | D<br>0.283 | E<br>0.444 |
| MOTOR OIL (10W30 viscosity grade) |            |            |            |            |            |
| ABSORBENT CAPACITY RETENTION      | 1:9.3      | 1:7.7      | 1:4.8      | 1:2.8      | 1:1.9      |
| ETHYLENE GLYCOL                   |            |            |            |            |            |
| ABSORBENT CAPACITY RETENTION      | medium     | medium     | medium     | medium     | weak       |
| HYDRAULIC FLUID                   |            |            |            |            |            |
| ABSORBENT CAPACITY RETENTION      | 1:9.1      | 1:7.4      | 1:4.4      | —          | —          |
| ACETONE                           |            |            |            |            |            |
| ABSORBENT CAPACITY RETENTION      | 1:6.8      | 1:5.6      | 1:3.3      | —          | —          |
|                                   | good       | good       | good       | —          | —          |

TABLE-continued

| 5       | DENSITY (g/cc)               | SAMPLES    |            |            |            |            |
|---------|------------------------------|------------|------------|------------|------------|------------|
|         |                              | A<br>0.077 | B<br>0.104 | C<br>0.176 | D<br>0.283 | E<br>0.444 |
| TOLUENE |                              |            |            |            |            |            |
| 10      | ABSORBENT CAPACITY RETENTION | 1:7.7      | 1:6.4      | 1:3.5      | —          | —          |

## DESCRIPTION OF TEST PROCEDURES

## Absorbent Capacity

The absorbent capacity test is used to determine the maximum amount of test liquid that a sample can pick-up. The test procedure comprises the following steps:

15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115

## 11

correlation between the density of the peat moss board and its absorbent capacity for the various non-aqueous liquids that are being used in the experiment. More particularly, it is apparent that by decreasing the density of the peat moss board, the absorbent capacity increases approximately in an exponential fashion. Accordingly, even a small density decrease can yield significant gains in absorption capacity. This is particularly true for density values below 0.2 g/cc.

The relationship between the density and the absorbent capacity is valid and confirmed for each test fluid. Although the absolute absorbent capacity changes according to the particular test fluid, the relationship is clearly observable in each case.

The results of the liquid retentivity test reported in the table demonstrate that the density of the peat moss board does not significantly affect its liquid retentivity. Rather, the ability of the peat moss board to prevent absorbed liquid from escaping the absorbent medium is largely dependent upon the nature of the liquid. For example, the peat moss board has a higher retentive power in connection with acetone and toluene than with regard to motor oil (viscosity grade 10 W 30), ethylene glycol and hydraulic fluid.

In use, to recover a spill of a certain non-aqueous liquid, the absorbent article in accordance with the invention is directly contacted with the liquid, such as by depositing the peat moss board in the spill, until the absorbent article is fully soaked with liquid. The spent absorbent article is then removed and treated in accordance with the applicable waste management techniques and regulations. The buoyancy and the ability of the absorbent article to block the penetration of water within the absorbent medium is advantageous for recovery operations conducted in an environment where large amounts of water are present, such as for example oil floating on sea surface. By dispersing on the water a sufficient number of absorbent articles to adequately cover the oil slick, the pollutant is collected within the peat moss boards which remain afloat even when soaked with liquid. As a result, the retrieval of the pollutant can be accomplished rapidly and in a cost-effective manner.

The scope of the present invention is not limited by the description, examples and suggestive uses herein as modifications and refinements can be made without departing from the spirit of the invention. Thus, it is intended that the present application covers the modifications and variations of this invention provided that they come within the scope of the appended claims and their equivalents.

We claim:

1. An absorbent article for collecting a non-aqueous liquid comprising a low density, hydrophobic, structurally integral board of peat moss material manifesting an affinity for the non-aqueous liquid, wherein said board of peat moss material is capable of absorbing the non-aqueous liquid under the effect of capillary pressure.

2. An absorbent article as defined in claim 1, wherein said board of peat moss material is oleophilic and capable of absorbing oil-based products.

3. An absorbent article as defined in claim 1, wherein said board of peat moss material has a density in the range from about 0.02 g/cc to about 0.20 g/cc.

4. An absorbent article as defined in claim 1, wherein said board of peat moss material has a density in the range from about 0.05 g/cc to about 0.15 g/cc.

5. An absorbent article as defined in claim 1, wherein said board of peat moss material has a density in the range from about 0.05 g/cc to about 0.10 g/cc.

6. An absorbent article as defined in claim 1, wherein said board of peat moss material has a laminated structure

## 12

including a reinforcing layer to enhance a structural integrity of said absorbent article.

7. An absorbent article as defined in claim 6, wherein said reinforcing layer forms an outer surface of said absorbent article.

8. An absorbent article as defined in claim 6, wherein said board of peat moss material includes an absorbent layer of peat moss material united in a face-to-face relationship with said reinforcing layer, said reinforcing layer being made of a fibrous material.

9. An absorbent article as defined in claim 8, wherein said board of peat moss material includes an upper reinforcing layer of fibrous material and a lower reinforcing layer of fibrous material, said absorbent layer of peat moss material being mounted between said upper and lower reinforcing layers of fibrous material.

10. An absorbent article as defined in claim 6, wherein said fibrous material is selected from the group consisting of Kraft wood pulp fibers, cotton linters, ground wood and mixtures thereof.

11. An absorbent article as defined in claim 1, wherein said board of peat moss material includes a component selected from the group consisting of polyester, nylon, acrylic, Kraft wood pulp, mechanical wood pulp, cotton linters, jute and mixtures thereof.

12. An absorbent article as defined in claim 1, wherein said board of peat moss material includes a water-repelling agent.

13. An absorbent article for recovering an oil-based liquid floating on a body of water, said absorbent article including a structurally integral and buoyant board of peat moss material, said board of peat moss material being hydrophobic and oleophilic, wherein when said board of peat moss material is floated on the body of water in contact with the oil-based liquid, said board of peat moss material selectively absorbs the oil-based liquid without taking-up any significant amount of water.

14. A method for manufacturing a low density, structurally integral article for collecting a non-aqueous liquid, said method comprising the steps of:

- forming a liquid suspension of peat moss material;
  - sheeting said suspension on a layer of fibers;
  - extracting fluidizing medium from said suspension to form a low density board of peat moss material to cause said fibers to adhere to said peat moss material;
  - drying said board of peat moss material at a temperature above 100° C. to evaporate residual moisture;
- said method being completed without conditioning said peat moss material with wetting agent to preserve a natural hydrophobicity of the peat moss material in order to impede water penetration in the article.

15. A method as defined in claim 14, comprising the step of forming an aqueous slurry of peat moss material to form said suspension.

16. A method as defined in claim 14, comprising the step of classifying said peat moss material to eliminate therefrom particles having a size smaller than 210 microns and particles having a size larger than 2000 microns.

17. A method as defined in claim 15, comprising the step of depositing over said suspension in sheeted form a layer of fibers, whereby the extraction of fluidizing medium from said suspension causes said fibers to adhere to said peat moss material.

18. A method as defined in claim 17, wherein said fibers are selected from the group consisting of Kraft pulp fibers, ground wood, cotton linters and mixtures thereof.

**13**

**19.** A method as defined in claim **14**, comprising the step of combining with said peat moss material a component selected from the group consisting of polyester, nylon, acrylic, Kraft wood pulp, mechanical wood pulp, cotton linters, jute and mixtures thereof.

**14**

**20.** A method as defined in claim **15**, comprising the step of treating said peat moss material and said layer of fibers with a water-repelling agent.

\* \* \* \* \*